

1

2,948,596

## NON-STALLING GASOLINE FUEL COMPOSITIONS

Henry A. Ambrose, Penn Township, Allegheny County, and Gardner E. Gaston, Tarentum, Pa., assignors to Gulf Research & Development Company, Pittsburgh, Pa., a corporation of Delaware

No Drawing. Filed Dec. 20, 1955, Ser. No. 554,142

4 Claims. (Cl. 44—58)

This invention relates to non-stalling gasoline fuel compositions that are adapted to improve the operation of internal combustion engines under cool, humid atmospheric conditions. More particularly, the invention relates to gasoline fuel compositions that contain a small amount, sufficient to reduce the tendencies of the composition to promote stalling in an internal combustion engine of the spark ignition, reciprocating type, of a salt of a dialkyl sulfosuccinic acid.

When an internal combustion engine is operated under cool, humid atmospheric conditions, using a gasoline fuel having a relatively low 50 percent ASTM distillation point, excessive engine stalling is apt to be encountered at idling speeds during the warm-up period, especially where engine idling occurs following a period of light load operation. Engine stalling under such conditions has been attributed to the partial or complete blocking of the narrow air passage that exists between the carburetor throat and the carburetor throttle valve during engine idling, by ice particles and/or solid hydrocarbon hydrates that deposit upon and adhere to the metal surfaces of the carburetor parts. Such icing of carburetor parts occurs as a result of the condensation of moisture from the air drawn into the carburetor and as a result of the solidification of such condensed moisture. The aforesaid condensation and solidification of moisture are caused by the refrigerating effect of rapidly evaporating gasoline. Accordingly, excessive engine stalling due to carburetor icing occurs as a practical matter only in the instance of gasolines containing a large proportion of relatively highly volatile components.

Excessive engine stalling is, of course, a source of annoyance owing to the resulting increased fuel consumption, battery wear and inconvenience of frequent restarting. It is therefore important that the inherent engine stalling characteristics of gasoline fuels be reduced substantially, where the 50 percent ASTM distillation point of such gasoline fuels is sufficiently low to cause a problem in this respect.

We have found that the stalling characteristics of gasoline fuel compositions having a 50 percent ASTM distillation point below about 220° F. and that normally tend to promote engine stalling due to carburetor icing are markedly improved by the incorporation therein of a small amount of a member selected from the group consisting of alkali metal, alkaline earth metal, ammonium, and ethyloammonium dialkyl sulfosuccinates, the alkyl groups of which each contain 7 to 9 carbon atoms, at least 6 of which are in a straight chain, but there being no group containing more than 7 carbon atoms attached to the alpha carbon atom of said alkyl groups. In one embodiment of the invention the gasoline composition also contains about 0.25 to about 0.75 percent by volume of the composition of a light lubricating oil having a viscosity at 100° F. of about 50 to about 500 Saybolt Universal seconds.

The dialkyl sulfosuccinate anti-stalling agents disclosed herein can be characterized as polar, surface-active ma-

2

terials. While the invention is not limited to any theory of operation, it might appear that the polarity of the disclosed agents tends to cause orientation of the latter upon the metal surfaces of the throttle valve and other critical carburetor parts contacted by the gasoline composition, thus forming a moisture-displacing, residual coating on said carburetor parts, which coating tends to prevent the adherence to said metal surfaces of accumulations of ice of magnitudes sufficient to block the narrow air passages that exist in carburetor throats at engine idling conditions. It is also considered that the dialkyl sulfosuccinates may orient themselves about small individual water or ice particles, thus tending to prevent the formation of macro-crystals of ice of a size sufficient to block carburetor air passages at engine idling conditions. Although the effectiveness of the herein disclosed addition agents is believed to be attributable at least in part to the polar characteristics thereof, this general explanation is somewhat negatived by the fact that many oil-soluble polar agents have little or no effect upon engine stalling due to carburetor icing.

When the herein disclosed dialkyl sulfosuccinate anti-stalling agents are utilized in gasoline compositions that contain a small amount of a light lubricating oil, it might appear that the dialkyl sulfosuccinates, by virtue of their affinity for the lubricating oil, tend to attract the oil to the same critical carburetor surfaces referred to above, while simultaneously increasing the spreading and metal wetting characteristics of the oil, thus promoting the formation of an adherent oil film on the metal surfaces of the carburetor parts. The oil film therefore would appear to function similarly as the dialkyl sulfosuccinates, but the superior metal wetting properties imparted to the oil by the additives are believed to enable the oil to displace moisture from metal carburetor surfaces that it would not thoroughly displace alone.

The preparation of the dialkyl sulfosuccinates disclosed herein is conventional and forms no part of the invention. However, in the interest of clarity, it may be generally mentioned that the dialkyl sulfosuccinates disclosed herein are conveniently prepared by esterification of maleic anhydride with a suitable monohydric alcohol, followed by addition to the resulting dialkyl maleate of a suitable bisulfite, for example, sodium bisulfite.

As indicated above, the present invention includes the use of alkali metal, alkaline earth metal, ammonium, and ethyloammonium salts of a particular class of dialkyl sulfosuccinic acids. This class of salts can be represented by the general formula:



where C, H, O and S are respectively carbon, hydrogen, oxygen and sulfur; where R is an alkyl group containing 7 to 9 carbon atoms, at least 6 of which are in a straight chain, there being no group attached to the alpha carbon atom of said alkyl groups containing more than 7 carbon atoms; where Z is a salt-forming group selected from the class consisting of alkali metal, alkaline earth metal, ammonium and ethyloammonium; and where n is an integer equal to the valence of Z. In the foregoing general formula, R can represent identical or different alkyl groups of the type specified above.

Especially effective results are obtained by the use of alkali metal dialkyl sulfosuccinates wherein the alkyl groups are branched and contain 8 carbon atoms, since the surface-active properties of such compounds appear to be less affected by low temperatures. An example of a dialkyl sulfosuccinate with which excellent results have

been obtained is the sodium salt of di-(2-ethylhexyl) sulfosuccinic acid, the formula of which is:



where Na is sodium and C, H, O, and S are as indicated above.

Examples of other dialkyl sulfosuccinates, the use of which is included by this invention, are the sodium, potassium, calcium, barium, ammonium and triethylolammonium salts of di-(n-heptyl), di-(n-octyl), di-(1-methylhexyl)-sec, di-(1-butylamyl)-sec, di-(isobutyl - 3 - methylbutyl)-sec, di-(2-ethylhexyl)-sec, di - (1-methylheptyl)-sec, and di-(1-methyl - 4 - ethylhexyl)-sec sulfosuccinic acids. Examples of salts of mixed esters that are suitable for the purposes of this invention are the sodium, potassium, calcium, barium, ammonium and triethylolammonium salts of mono-2-ethylhexyl, mono-1-methyl-4-ethylhexyl sulfosuccinic acid, and mono-2-ethylhexyl, mono-1-methylheptyl sulfosuccinic acid.

The class of dialkyl sulfosuccinates included by this invention possess a substantially similar balance of surface-active properties, as a result of which they are rendered suitable for the purposes of this invention. The similarity in the surface-active properties of the dialkyl sulfosuccinates included in the scope of this invention is evidenced by the fact that the class of compounds disclosed exhibit relatively low water solubility and unusually low Draves wetting power values. In general, the Draves wetting power value for the class of dialkyl sulfosuccinates included by the invention will not substantially exceed about 0.5 while the preferred class of materials will exhibit Draves wetting power values between about 0.15 and about 0.25. In contrast, dialkyl sulfosuccinates whose alkyl groups and/or salt-forming groups are other than as defined herein will exhibit Draves wetting power values substantially in excess of the maximum indicated above, and they will also normally exhibit substantially greater solubility in water. It is understood, of course, that the foregoing discussion is not necessarily intended to suggest any direct connection between water solubility or wetting power and anti-stalling characteristics. Rather, it is intended merely to indicate the similar, over-all balance of surface-active properties possessed by the class of compounds disclosed herein as useful. The specific Draves wetting power values given above refer to the number of grams per liter required to give a 25 second sinking time by the Draves test at 30° C. The Draves test is a conventional test for determining wetting power.

The dialkyl sulfosuccinate anti-stalling agents described herein are useful when incorporated in gasoline compositions of the type disclosed in an amount sufficient to reduce the engine stalling characteristics thereof. For example, an improvement in the stalling characteristics of gasolines of the type disclosed will normally be obtained by the addition thereto of the herein disclosed dialkyl sulfosuccinates in amounts of at least 0.001 percent by weight of the composition, i.e., about 3 pounds per thousand barrels of gasoline. For fully effective results, the dialkyl sulfosuccinate anti-stalling agents disclosed herein will be employed in proportions of at least about 0.005 percent by weight of the composition, i.e., about 15 pounds per thousand barrels of gasoline. Excellent results have been obtained by the addition of a dialkyl sulfosuccinate of the kind disclosed herein to gasoline compositions in proportions between 15 and 50 pounds per thousand barrels of gasoline, and this constitutes the preferred concentration range for the purposes of this invention. However, larger proportions can be used.

In most instances the concentration of the herein disclosed anti-stalling agents need not exceed about 0.1 percent by weight of the composition, even in instances of gasolines having severe engine stalling tendencies.

- 5 It will be appreciated that the optimum concentration of the disclosed dialkyl sulfosuccinate anti-stalling agents can vary within the disclosed range according to the particular gasoline employed, since the problem of engine stalling due to carburetor icing is a function of the 50 percent ASTM distillation point of the gasoline. Thus, greater concentrations of the additive are normally desirable with decreasing 50 percent ASTM distillation point. The optimum concentration of the dialkyl sulfosuccinate anti-stalling agents can also vary somewhat according to the particular make and model of engine in which the gasoline is used and also according to the severity of the atmospheric conditions encountered. With regard to the last mentioned factor, the problem of engine stalling due to carburetor icing resulting from the refrigeration by evaporating gasoline of moisture condensed from the atmosphere has been observed to be significant at temperatures between about 30° and 50° F., e.g., 35°, 40°, 45°, 50° F., and when the relative humidity is in excess of about 65 percent, e.g., 75, 85, 99 percent.
- 10 25 The optimum concentration of the dialkyl sulfosuccinate anti-stalling agents will be one that is sufficient to effect a substantial reduction in the stalling tendencies of the fuel at the atmospheric conditions of temperature and humidity which are likely to be encountered in service.
- 30 35 Practically speaking, the problem of engine stalling due to carburetor icing caused by rapid evaporation of gasoline occurs only in connection with gasolines having a 50 percent ASTM distillation point of not greater than about 235° F. While occasional engine stalling may occur as a result of carburetor icing at severe atmospheric conditions of temperature and humidity with gasolines having somewhat higher 50 percent ASTM distillation points, experience has indicated that the problem does not assume major importance except with gasolines of the character indicated. The problem of engine stalling due to carburetor icing is especially severe in connection with gasolines having a 50 percent ASTM distillation point of less than about 220° F. The invention is particularly useful in connection with such gasolines. The term "gasoline" is used herein in its conventional sense to include hydrocarbon mixtures having a 90 percent ASTM distillation point of not more than about 392° F. and a 10 percent ASTM distillation point of not more than about 140.
- 40 45 50 As previously indicated, the gasoline compositions of this invention are additionally benefited with respect to non-stalling characteristics by the inclusion therein of a small amount of a lubricating oil having a viscosity at 100° F. of between about 50 and about 500 Saybolt 55 Universal seconds; for example, an oil having a viscosity of about 100 S.U./100° F. can be used with advantage. Although highly paraffinic lubricating distillates can be used, lubricating distillates obtained from Coastal or naphthenic type crude petroleum oils are preferred because of their superior solvent properties. The lubricating oils utilized in the gasoline compositions of this invention can have been solvent-treated, acid-treated or otherwise refined prior to incorporation into the gasoline compositions of this invention. The lubricating distillates referred to are useful in the gasoline compositions of this invention in amounts of from about 0.25 to about 0.75 percent by volume of the composition, for example 0.5 volume percent. In such concentrations these lubricating distillates tend to assist the anti-stalling function of the dialkyl sulfosuccinates and in addition as cleansing solvents and as upper cylinder and valve top lubricants. Greater amounts of lubricating oil can be used but without appreciable further improvement in the stalling tendencies of the gasoline composition; however, the amount of lubricating oil used should

not be so great as to adversely affect the volatility and combustion characteristics of the ultimate gasoline compositions.

The dialkyl sulfosuccinate anti-stalling agents of this invention can be incorporated into the base gasoline fuel compositions in any suitable manner. Thus, they can be added as such to gasoline or in the form of a dispersion or solution in solvents such as butanol, isopropanol, ethanol, methanol, 2-butoxyethanol, diethylene glycol monobutyl ether, benzene, toluene, heptane, kerosene, gasoline, mineral oil or the like, which solvents may or may not themselves additionally contribute to the anti-stalling characteristics of the ultimate composition. If desired, the disclosed dialkyl sulfosuccinate anti-stalling agents can be incorporated in gasoline fuel compositions in admixture with other materials designed to improve one or more properties of the gasoline such as antioxidants, anti-gumming agents, anti-knock agents, e.g., tetraethyl lead, lead scavenging agents, e.g., ethylene dibromide, ignition control additives, de-icing agents, corrosion inhibitors, dyes and the like.

Gasoline compositions of this invention can be further illustrated by the following representative specific examples.

#### EXAMPLE I

A motor gasoline composition according to this invention and having reduced engine stalling tendencies was prepared by incorporating sodium di-(2-ethylhexyl) sulfosuccinate, in the proportion of 15 pounds per thousand barrels, in a sample of motor gasoline having a strong tendency as such to promote engine stalling due to carburetor icing. The base gasoline employed in this example was a blend containing 12 parts by volume of a light thermally cracked gasoline distillate and 100 parts by volume of a gasoline distillate having the following inspections:

|                                |      |
|--------------------------------|------|
| Gravity, ° API                 | 64.4 |
| Anti-knock rating, Octane No.: |      |
| Motor Method                   | 79.3 |
| Research Method                | 82.8 |
| TEL, ml./gal                   | 2.96 |
| Vapor pressure, Reid, lb.      | 7.0  |
| Distillation, gasoline:        |      |
| Over point, ° F                | 106  |
| End point, ° F                 | 388  |
| 10% evap. at ° F               | 145  |
| 50%                            | 206  |
| 90%                            | 287  |

The blended gasoline had a 50 percent distillation point of 200° F.

#### EXAMPLE II

An additional motor gasoline composition in accordance with this invention and having reduced engine stalling characteristics was prepared by admixture of sodium di-(2-ethylhexyl) sulfosuccinate, in the proportion of 15 pounds per thousand barrels of gasoline, with the blended base gasoline described in Example I, to which there was also added 0.5 percent by volume of an approximately 100 S.U.S./100° F. Texas (Coastal) lubricating distillate, a sample of which had the following inspections:

|                                    |      |
|------------------------------------|------|
| Gravity, ° API                     | 24.5 |
| Viscosity, SUV, sec.:              |      |
| 70° F                              | 235  |
| 100° F                             | 106  |
| 130° F                             | 63.9 |
| 210° F                             | 38.3 |
| Viscosity index                    | 16   |
| Pour, ° F                          | 60   |
| Carbon residue, Conradson, percent | 0.02 |

The foregoing specific embodiments of the compositions of this invention are illustrative, and other suitable

compositions within the scope of this invention and having satisfactory anti-stalling characteristics can be prepared similarly by the substitution in the foregoing examples of other gasolines of the type disclosed herein and by the incorporation therein of the same or equivalent proportions within the range disclosed of the dialkyl sulfosuccinates disclosed herein. For example, good results can be obtained by incorporation in the blended base gasoline of Example I 50 pounds, per thousand barrels of gasoline, of the sodium, potassium, calcium, barium, ammonium and triethylolammonium salts of di-(n-heptyl), di-(n-octyl), di-(1-methylhexyl)-sec, di-(1-butylamyl)-sec, di-(isobutyl-3-methylbutyl)-sec, di-(2-ethylhexyl)-sec, di-(1-methylheptyl)-sec, and di-(1-methyl-4-ethylhexyl)-sec sulfosuccinic acids.

As heretofore indicated, the dialkyl sulfosuccinate anti-stalling agents of this invention produce an appreciable improvement in the stalling characteristics of gasolines that normally promote engine stalling due to carburetor icing. To illustrate the nature of the improvement obtained, in the table following there are presented illustrative results obtained with engine tests using a gasoline fuel composition prepared in accordance with this invention. For purposes of comparison there are also presented in the table below the results obtained with engine tests carried out on a sample of the uninhibited test gasoline.

According to the test procedure followed the fuel compositions to be tested were fed to a standard, 216 cubic inch displacement, 6-cylinder overhead valve Chevrolet engine, the air supply to the carburetor of the engine being obtained by natural aspiration from a cold room atmosphere. The engine was equipped with a standard Carter downdraft carburetor. The ambient temperature of the cold room was 40° F., and the relative humidity was 80 to 85 percent.

The first operating cycle of the engine included, after permitting the engine to cool to the ambient temperature of 40° F., starting the engine and running for 40 seconds at 2000 r.p.m. and then for 20 seconds at 500 r.p.m. (idle) under no load, or until the engine stalls. Repetition of the foregoing cycle 20 times constituted one test.

Table

| Composition | Base Fuel                                                                 | Additive                                                      | Concentra-tion, Lbs./1000 Bbls. | Engine Test: Stalls Per 20 Operating Cycles |
|-------------|---------------------------------------------------------------------------|---------------------------------------------------------------|---------------------------------|---------------------------------------------|
| 1           | Base Gasoline, 200° F. 50% ASTM Distillation Point (Example I Base Fuel). |                                                               |                                 | 11 (avg., 12 tests).                        |
| 2           | Base Gasoline.                                                            | Sodium Di-(2-ethylhexyl) Sulfosuccinate (Example I Additive). | 15                              | 2.3 (avg., 3 tests).                        |
| 3           |                                                                           |                                                               |                                 |                                             |

From the results presented in the foregoing table it will be seen that uninhibited gasolines having a 50 percent ASTM distillation point in the range disclosed possessed poor stalling characteristics. In tests of other uninhibited base fuels it was found that a gasoline having a 50 percent ASTM distillation point of 230° F. produced an average (7 tests) of 1.4 stalls, whereas a gasoline having a 50 percent ASTM distillation point of 240° F. produced an average (19 tests) number of stalls approaching zero. From the data in the foregoing table it is also apparent that gasolines having a 50 percent ASTM distillation point within the range disclosed herein will be markedly improved by incorporation therein of the

herein disclosed proportions of the dialkyl sulfosuccinate anti-stalling agents of this invention.

To the gasoline fuel compositions of this invention there can also be added one or more additional additive agents designed to improve one or more characteristics of the gasoline fuel. For example, antioxidants, anti-knock agents, ignition control agents, other deicing agents, anti-rust agents, dyes, lead scavenging agents, anti-gumming agents and the like can be added to the compositions of this invention, and the invention specifically includes gasoline compositions containing such additives.

Numerous additional embodiments of the invention will readily suggest themselves to those skilled in the art. Accordingly, we do not intend to be limited by the foregoing description, but only by the terms of the claims appended hereto.

We claim:

1. A gasoline fuel composition comprising a major amount of a hydrocarbon mixture that boils in the gasoline range, that has a 50 percent ASTM distillation point not greater than about 220° F. and that normally tends to promote stalling of internal combustion engines, and containing a combination of (a) 0.001 to about 0.1 percent by weight of the composition of a member selected from the group consisting of alkali metal, alkaline earth metal, ammonium and ethyl ammonium salts of dialkyl sulfosuccinic acids, the alkyl groups of which each contain 7 to 9 carbon atoms, at least 6 of which are in a straight chain, no group attached to the alpha carbon atom of said alkyl groups containing more than 7 carbon atoms, and (b) about 0.25 to about 0.75 percent by volume of the composition of a light lubricating oil having a viscosity at 100° F. of about 50 to about 500 S.U.S., the amount of said combination being sufficient to reduce the engine stalling characteristics of the gasoline composition.

2. A gasoline fuel composition comprising a major amount of a hydrocarbon mixture that boils in the gasoline range, that has a 50 percent ASTM distillation point not greater than about 220° F. and that normally tends to promote stalling of internal combustion engines, and containing a combination of (a) 15 to 50 pounds, per thousand barrels of said hydrocarbon mixture, of sodium di-(2-ethylhexyl) sulfosuccinate, and (b) about 0.25 to about 0.75 percent by volume of the composition of a light lubricating oil having a viscosity at 100° F. of about 50 to about 500 S.U.S., the amount of said combination

of oil and sodium di-(2-ethylhexyl) sulfosuccinate being sufficient to reduce the engine stalling characteristics of the gasoline composition.

3. A gasoline fuel composition comprising a major amount of a hydrocarbon mixture that boils in the gasoline range, that has a 50 percent ASTM distillation point not greater than about 220° F. and that normally tends to promote stalling of internal combustion engines, and containing a combination of (a) about 15 pounds, per thousand barrels of said hydrocarbon mixture, of sodium di-(2-ethylhexyl) sulfosuccinate, and (b) about 0.5 percent by volume of a light lubricating oil having a viscosity at 100° F. of about 50 to about 500 S.U.S., the amount of said combination of oil and sodium di-(2-ethylhexyl) sulfosuccinate being sufficient to reduce the engine stalling characteristics of the gasoline composition.

4. A gasoline motor fuel composition comprising a major amount of a motor gasoline that has a 50 percent ASTM distillation point not greater than about 220° F. and that normally tends to promote stalling of automotive internal combustion engines, and containing a combination of (a) 15 to 50 pounds per thousand barrels of gasoline of sodium diethylsulfosuccinate, and (b) about 0.25 to about 0.75 percent by volume of the composition of a light lubricating oil having a viscosity at 100° F. of about 50 to about 500 S.U.S., the amount of said combination of oil and sodium diethylsulfosuccinate being sufficient to reduce the engine stalling characteristics of the gasoline composition.

30

#### References Cited in the file of this patent

#### UNITED STATES PATENTS

|           |                       |               |
|-----------|-----------------------|---------------|
| 2,316,739 | Cook et al. -----     | Apr. 13, 1943 |
| 2,548,630 | Sorg et al. -----     | Apr. 10, 1951 |
| 2,550,982 | Eberz -----           | May 1, 1951   |
| 2,600,113 | Jones et al. -----    | June 10, 1952 |
| 2,668,522 | Hickok et al. -----   | Feb. 9, 1954  |
| 2,706,677 | Duncan et al. -----   | Apr. 19, 1955 |
| 2,851,343 | Cantrell et al. ----- | Sept. 9, 1958 |

#### OTHER REFERENCES

"Aviation Gasoline Manufacture," by Van Winkle, McGraw-Hill Co., N.Y., 1944, First Ed., pp. 16 and 17.

"ASTM" Standards on Petroleum Products and Lubricants, American Society for Testing Materials, November 1955, p. 370.